

## UNITED STATES PATENT OFFICE

2,542,716

## MULTICOLOR DIAZOTYPE LAYERS

Sam Charles Slifkin, Binghamton, N. Y., assignor  
to General Aniline & Film Corporation, New  
York, N. Y., a corporation of Delaware

No Drawing. Application December 5, 1947, Se-  
rial No. 790,026. In Great Britain July 16, 1945

5 Claims. (Cl. 95—6)

1

This invention relates to diazotype light sensitive media. More particularly, it relates to that type of diazotype reproduction media wherein the positive copies obtained from the exposure of the reproduction media under a positive original is developed in the dry state by contact with a gaseous developing agent. This application is a continuation-in-part of my copending application Serial No. 545,201, filed July 15, 1944, now abandoned.

Diazotypes of this class are generally produced by treating the surface of a suitable base such as paper, cellulose acetate film, cellophane, glass and metal surfaces with a solution of two dye components, one of which, the diazo compound, is the photosensitive body and the other, the azo component or coupling component, is a compound capable of reacting under suitable conditions with the diazo compound to form a dye. The diazo compound will decompose, upon exposure to light, particularly light which emits rays in the 3600 Å. to 4200 Å. line, to form a compound which can no longer combine with the azo coupling component. This decomposition product, however, may itself be a coupling component and may be employed in some instances to combine with undecomposed diazo compound.

When a diazotype layer containing a diazo compound and a coupling component is exposed under an original tracing, design or printed sheet to a proper source of light, the diazo compound, in those areas which are not protected by the solid lines of the tracing or design or letters of the printed sheet, is decomposed. Upon subsequent development, a dye forms only in the areas which were protected from the light by the said lines of the tracing, design or letters of the printed sheet and thus the original is reproduced in the color called for by the particular combination of a diazo compound and coupling component present in the light sensitive layer. In cases where there is a distinct variation in the densities of various parts of the original which is to be copied, such as where there are ink lines and pencil marks or pencil lines on the same original drawing or where there are shadows and high-lights on a design, the lines of weaker density, half-tones or high-lights will appear, if at all, as indistinct or dispersed shades of the same color tone as the full densities or shadows. In many cases where the contrast between the full

2

densities and the half-tones or high-lights of the original is very great, no reproduction of the half-tones or high-lights will be obtained since the degree of exposure necessary to decompose the diazo compound in the background areas will also completely or almost completely decompose the diazo compound in the half-tone or high-light areas.

It has now been discovered that the full densities or shadows and the half-tones or high-lights of an original can be reproduced in different colors, thus indicating the existing difference in densities without the necessity of creating such a low density in the reproduction of the half-tones or high-lights as to render them indistinct. This effect is produced by adding to the light sensitive coating solution a number of coupling components differing widely from each other in their coupling rates or potentials and forming contrasting colors when coupled with the diazo compound.

It has been observed that the rate of formation of an azo dye is dependent upon many variables but is in large part predetermined by the inherent nature of the diazonium compound and the coupler or couplers used in the formation of the azo dye. Thus, under identical conditions, a single diazo compound will couple at greatly varying rates with a series of different azo components or couplers and a single coupling component will also couple at greatly varying rates with a series of different diazo compounds. Thus, in the selection of diazo compounds and couplers for the production of a diazotype light sensitive layer, the combination of a slow coupling diazo and a fast coupling azo component will be similar in effect to a fast coupling diazo and a slow coupling azo component. This effect produced by the inherent properties of the diazo compound and coupling component is referred to as the coupling potential and wherever that term is used throughout this specification and appended claims, it will be understood therefore to mean the coupling time-relation between a given diazo compound and a given coupling component.

This variation in the coupling potentials in a diazotype system containing a single diazo compound and two or more coupling components is the controlling factor in the selectivity of the diazo for the coupler determining the color of

a given density area. The relative concentration of the coupling components is also a contributing factor. Thus, concentration can be used to offset the unfair competition of the more energetic coupler having a higher coupling potential. In areas where there is a high concentration of diazo the coupler of high coupling potential will be used up first. Then coupling will take place with the less energetic coupler. By limiting the concentration of the high potential coupler the color produced by the slow coupler will predominate in such areas of high diazo concentration.

When using a continuous tone or multi-density original the concentration of the light sensitive diazo is varied by exposure to light of a diazotype under such an original so that a series of different concentrations of diazo are produced on the irradiated sheet. The concentration of the couplers in a two-component diazotype system will remain the same throughout. In each density area of the exposed diazotype then will be competitive coupling controlled by the coupling potentials and relative concentrations of the couplers. By using a relatively high concentration of the slower coupler and a relatively small amount of the fast coupler, coupling will be controlled by the energetic coupler only in the areas where there is a low concentration of the diazo. The diazo in those areas will become exhausted by the energetic coupler before the slow coupler has an opportunity to exert its influence. As the concentration of the diazo increases in the half-tone areas, where there is not enough of the energetic coupler to combine with all of the residual diazo, more and more of the slow coupler will react until in the high density areas the slow coupler exerts its influence on the color produced to its fullest extent. Any color produced by the energetic or fast coupler in such areas will be completely overshadowed by the color of the slow coupler.

In order to obtain optimum contrast between the high density and low density areas it is preferable to not only react a combination of energetic and slow couplers which will produce contrasting colors with the diazo compound, but to combine the couplers in such a molar ratio to each other that the slow coupler will be in considerable excess. The exact ratio will depend upon the tintorial strength of the color produced by the slow coupler, there being sufficient of the more active or energetic coupler present to prevent any appreciable degree of coupling by the slow coupler in the half-tones or highlight areas. Ratios of from  $1/10$  to  $1/40$  in favor of the slow coupler have been found satisfactory.

Diazo compounds which are most suitable for the production of the dual tone or multicolor effects of this process are those which are derived from p-diamines of the benzene series. Examples of such diazo compounds are p-diazo-N-diethyl-m-toluidine; p-diazo-diphenylamine; p-diazo-N-diethylaniline; p-diazo-N-methylaniline; p-diazo-N-dimethylaniline; p-diazo-N-ethoxyaniline; p-diazo-N-ethyl-N-ethoxyaniline; 1-diazo-3-methyl-4-N-ethylaminobenzene; and 1-diazo-3-methoxy-4-N-cyclohexylaminobenzene. These diazo compounds are preferably used in the form of their double salt complexes, such as the zinc chloride double salt, the cadmium chloride double salt, the chlorobenzenesulfonate, the tin chloride double salt, the borofluoride and the sulfate of the diazo compound.

This invention will be more fully understood

from the following examples which are illustrative of the invention but are not intended to limit in any way the scope thereof. The parts are by weight unless otherwise specified.

#### Example I

A coating solution is prepared by slowly mixing the following ingredients in the proportions given at room temperature:

|    |                               |    |      |
|----|-------------------------------|----|------|
| 10 | Water                         | cc | 80   |
|    | Glycerin                      | cc | 5    |
|    | Citric acid                   | g  | 10   |
|    | Zinc chloride                 | g  | 5    |
| 15 | Thiourea                      | g  | 5    |
|    | m-Hydroxy phenylurea          | g  | 1    |
|    | 2,3-dihydroxy naphthalene     | g  | 0.05 |
|    | p-Diazo diphenylamine sulfate | g  | 5    |

20 A diazotype stock paper is coated with the above solution in the usual manner by employing a doctor blade to remove the excess solution and the thus coated paper is then dried. Samples of this coated paper may then be exposed to light under a diapositive containing full density and half-tone areas and the thus exposed sensitized samples developed in the usual manner by contacting the sensitized side of the paper with a mixture of water vapor and ammonia gas. The 25 full density areas of the original will be reproduced in a green tone and the half-tone or low density areas will be reproduced in a purple tone. If 2 grams of the m-hydroxy phenylurea coupler instead of 1 gram are used in the coating solution 30 of this example, the reproduction in the full density areas will be in a yellow-green tone and that in the lower density areas in a bluish-black tone.

#### Example II

A coating solution is prepared by slowly mixing the following ingredients in the proportions given at room temperature:

|    |                               |    |      |
|----|-------------------------------|----|------|
| 45 | Water                         | cc | 80   |
|    | Glycerin                      | cc | 5    |
|    | Citric acid                   | g  | 10   |
|    | Zinc chloride                 | g  | 5    |
|    | Thiourea                      | g  | 5    |
| 50 | 2,3-dihydroxy naphthalene     | g  | 0.05 |
|    | 7-hydroxy-1,2-naphthimidazol  | g  | 1    |
|    | p-Diazo-N-diethyl aniline     | g  |      |
|    | ZnCl <sub>2</sub> double salt | g  | 3    |

55 A diazotype stock paper is coated with the above solution in the usual manner by employing a doctor blade to remove the excess solution and the thus coated paper is then dried. Samples of this coated paper may then be exposed to light under a diapositive having full density and half-tone areas and the thus exposed samples developed by contacting the sensitized side of the paper with a mixture of water vapor and ammonia gas. The full density areas of the original will be reproduced in a red tone and the half-tone or low density areas will be reproduced in a blue tone. If  $\frac{1}{2}$  gram of the 7-hydroxy-1,2-naphthimidazol coupler is used instead of 1 gram in the coating solution of this example, the full density areas will be reproduced in a red-purple tone and the low density areas in a blue tone.

75 The following table provides further combinations of slow and fast couplers which will give contrasting colors with the diazo compound, it being understood that the coating composition is prepared in the same manner as given above

in Examples I and II, the slow coupler being always used in excess ratio over the fast coupler.

6 areas of an original in contrasting colors which comprises in combination a mono-diazo deriva-

| Diazo Compound            | Slow Coupler                                       | Fast Coupler                            | Color of High Density Areas | Color of Low Density Areas |
|---------------------------|----------------------------------------------------|-----------------------------------------|-----------------------------|----------------------------|
| p-diazo-diphenyl-amine    | m-hydroxy-acetanilide                              | 2,3-dihydroxy-naphthalene               | Green                       | Blue                       |
| p-diazo-N-diethyl aniline | 7-hydroxy-naphthalene-1,2-imidazole                | 1,8-dihydroxy-naphthalene-sulfonic acid | Red                         | Do                         |
| p-diazo-diphenyl-amine    | m-hydroxy-phenylurea                               | 2,3-dihydroxy-naphthalene               | Green                       | Purple                     |
| p-diazo-N-diethyl aniline | 7-hydroxy-naphthalene-1,2-imidazole                | do                                      | Red                         | Blue                       |
| Do                        | 2-hydroxy-3-naphthoic acid (ethylenediamine amide) | phenylmethyl pyrazolone                 | Blue                        | Red                        |
| Do                        | 7-hydroxy-naphthalene-1-biguanide                  | Orcinol                                 | Purple/Black                | Red/Brown                  |

Having now particularly set forth and described my invention and having illustrated the best method of performing it, what I now claim as new is:

1. A diazotype light sensitive layer for the reproduction of different photographic density areas of an original in contrasting colors which comprises in combination a monodiazo derivative of a p-diamine of the benzene series and, in the ratio of from 1/10 to 1/40 by weight, a fast coupling component selected from the group consisting of 2,3-dihydroxynaphthalene, 1,8-dihydroxynaphthalene-4-sulfonic acid, phenylmethyl pyrazolone and orcinol and a slow coupling component selected from the group consisting of m-hydroxyacetanilide, m-hydroxyphenylurea, 7-hydroxynaphthalene-1,2-imidazole, ethylenediamine amide of 2-hydroxy-3-hydroxy-3-naphthoic acid and 7-hydroxynaphthalene-1-biguanide, the said slow coupling component being so selected as to produce with the diazo compound a different color tone than is produced by combination of the diazo compound with the fast coupling component.

2. A diazotype light sensitive layer for the reproduction of different photographic density areas of an original in contrasting colors which comprises in combination a monodiazo derivative of a p-diamine of the benzene and, in the ratio from 20/1 to 40/1 by weight, m-hydroxyphenylurea, and 2,3-dihydroxynaphthalene.

3. A diazotype light sensitive layer for the reproduction of different photographic density areas of an original in contrasting colors which comprises in combination p-diazo-diphenylamine, and, in the ratio of 20/1 by weight, m-hydroxyphenylurea, and 2,3-dihydroxynaphthalene.

4. A diazotype light sensitive layer for the reproduction of different photographic density

tive of a p-diamine of the benzene series and, in the ratio from 10/1 to 20/1 by weight, 7-hydroxynaphthalene-1,2-imidazol, and 2,3-dihydroxynaphthalene.

5. A diazotype light sensitive layer for the reproduction of different photographic density areas of an original in contrasting colors which comprises in combination p-diazo-N-diethylaniline and, in the ratio of 20/1 by weight, 7-hydroxynaphthalene-1,2-imidazol, and 2,3-dihydroxynaphthalene.

SAM CHARLES SLIFKIN.

#### REFERENCES CITED

The following references are of record in the file of this patent:

#### UNITED STATES PATENTS

| Number    | Name           | Date          |
|-----------|----------------|---------------|
| 1,760,780 | Schmidt et al  | May 27, 1930  |
| 1,845,989 | Schmidt et al. | Feb. 16, 1932 |
| 1,966,755 | D'Hauterine    | July 17, 1934 |
| 1,967,351 | Schmidt et al. | July 24, 1934 |
| 1,989,065 | Schmidt et al. | Jan. 22, 1935 |
| 2,034,508 | De Boer et al. | Mar. 17, 1936 |
| 2,037,542 | Schmidt et al. | Apr. 14, 1936 |
| 2,095,408 | De Boer et al. | Oct. 12, 1937 |
| 2,150,565 | Schmidt et al. | Mar. 14, 1939 |
| 2,157,206 | Hinman         | May 9, 1939   |
| 2,381,984 | Reichel        | Aug. 14, 1945 |

#### FOREIGN PATENTS

| Number  | Country | Date          |
|---------|---------|---------------|
| 660,087 | France  | Feb. 12, 1929 |

#### OTHER REFERENCES

Spencer: "Photographic Application of Diazo Compounds," The Photographic Journal, London, Dec. 1928, pp. 490 to 496.